

Aug. 11, 1942.

C. T. GORDON

2,292,369

METHOD OF PRODUCING ANTSILIP SURFACES FOR BATH FLOORS

Original Filed Oct. 19, 1939



Fig. 1.



Fig. 2.



Fig. 3.



Fig. 5.



Fig. 4.

INVENTOR  
CHARLES T. GORDON  
BY *John L. Milton*  
ATTORNEY

## UNITED STATES PATENT OFFICE

2,292,369

## METHOD OF PRODUCING ANTI-SLIP SURFACES FOR BATH FLOORS

Charles T. Gordon, Louisville, Ky., assignor to  
Porcelain Metals Corporation of Louisville,  
Kentucky, Louisville, Ky., a corporation of  
Kentucky

Original application October 19, 1939, Serial No.  
300,178. Divided and this application August  
12, 1940, Serial No. 352,260

## 3 Claims. (Cl. 41—24)

This application is a division of my earlier application Serial No. 300,178 filed October 19, 1939, and entitled "Vitreous enamel bath floor," and the invention disclosed herein relates to the method of producing the anti-slip floor-surface for the shower receptor disclosed in my aforesaid application.

The principal object of this invention is to provide a process of applying and firing vitreous enamel on the floor surface of a receptor so as to produce an anti-slip vitreous-surface.

Another object of this invention is to provide a process of producing an anti-slip vitreous-surface having raised areas of unglazed vitreous-enamel upon a glazed surface of vitreous-enamel.

A further object of this invention is to provide a process of producing an anti-slip vitreous-surface having a plurality of small areas coated with a granular material fused to the outer-surface of a glazed vitreous-enamel surface.

These and other objects will manifest themselves as the following description is read in connection with the accompanying drawing, in which:

Figure 1 is a plan view of a receptor illustrating traction areas 13 applied to a glazed vitreous-surface 14 by the method disclosed herein;

Figure 2 is a sectional view taken along lines 2—2 of Figure 1 illustrating the raised relation of the traction areas 13 relative to the glazed vitreous-surface 14;

Figure 3 is an enlarged sectional view taken along lines 3—3 of Figure 1 illustrating the amalgamation of the liquified frit or frits of the glazed coating 14 and the partially liquified frit or frits of the traction coating 13 along a mutual margin 15.

Figure 4 is a partial plan view of a receptor illustrating a modified arrangement of the traction areas, which arrangement may also be made by the method disclosed herein;

Figure 5 is a partial sectional view taken along lines 5—5 of Figure 4.

Shower-bath cabinets, to which the present invention has particular application, have gained quite extensive use. Accordingly, the slipperiness of the vitreous-enamel surface of the floor has become an important consideration. Heretofore, the entire surface of the floor has been made rough, somewhat like the surface of sandpaper, by sprinkling dry sand into the wet frit applied for the glazed finish-coat. However, by reason of this depositing of the sand into a wet frit, considerable care was required to avoid a glazing-over of the sand when firing the frit of the glazed

finish-coat. Further, because of the relative overall coarseness of the floor-surface, it was difficult to maintain clean and sanitary. Thus, it is the purpose of this invention to provide a process of applying and firing vitreous-enamels on the floor surface of a receptor, so as to provide an antislipping floor-surface having improved operating characteristics and advantages.

In the following description, the expression "traction-spot" is employed to designate the relatively small areas on the surface of the floor that will have a dull, matte or granular surface, which areas provide the required traction or "non-slip" characteristics for the glazed-surface of the floor.

Before describing the steps of the method by which the antislip floor-surface is produced, a short resume of the article embraced by the application referred to at the outset will be made.

In the accompanying drawing, the numeral 10 designates a floor of a receptor for a shower-bath cabinet, which floor has a perimetrical flange 12 projecting vertically therefrom. As illustrated in Figure 2, the floor 10 is depressed, and has a central aperture 11, which aperture provides a suitable drain outlet for waste water.

In Figure 1, the numeral 14 designates a glazed, vitreous-enamel surface, which surface completely covers the floor of the receptor, except as interrupted on its exposed outer-surface by elevated traction-spots 13. In the embodiment illustrated in Figure 1, the traction areas are illustrated as having a diamond shape, and are arranged in rows extending radially outwardly from the central drain 11.

Each of the diamond-shaped traction-spots 13 are elevated relative to the glazed, vitreous-enamel surface 14, and are constructed and arranged so that waste water will drain rapidly therefrom onto the glazed, vitreous-enamel surface 14.

Therefore, it is to be understood that the method described later in detail, may be employed to provide any desired pattern or design for the raised traction spots. It is also emphasized that, although the method is described as having particular reference to a receptor of a shower-bath cabinet, the method may be employed to provide a non-slip floor surface for other bathing appliances such as conventional bath tubs, etc.

Thus, the floor surface of bathing appliances produced in accordance with the foregoing method are made advantageously slip-proof of uniformly distributing traction-spots over the glazed-surface thereof in accordance with a predeter-

mined plan, which traction-spots are permanently anchored in the enamel of the glazed-surface. Accordingly, such floors are permanent, adequately slip-proof, and relatively easy to maintain clean.

To produce the non-slip floor-surface, the invention contemplates using two enamel frits, one of which has a maturing temperature higher than the other. The frit having the lower maturing temperature is first applied to the entire surface of the floor, and then the frit having the higher maturing temperature is deposited on top of the first frit in the form of the desired pattern. Both frits are then fired at the required temperature and for a time sufficient to mature the first frit, which temperature and time is appreciably less than that required to mature the second frit. Thus, the first frit is completely matured, and has a highly glazed surface, while the second frit is not matured and has a uniform dull or matte finish.

Some latitude may be exercised in regards to the firing temperature. Therefore, if desired, the firing temperature may be higher than that indicated in the preceding paragraph, but less than the maturing temperature of the second frit, under which condition the frits are fired for a time sufficient only to mature completely the first frit into a highly glazed surface, and stopped before the second frit matures or settles appreciably into the molten body of the first frit.

Thus, it will be apparent that the invention contemplates applying the two frits separately, so that the unmatured second frit will remain elevated relative to the matured first frit. Accordingly, since the matured first frit provides a highly glazed-surface and the unmatured second frit provides a dull or matte surface, the dull or matte surface of the traction spots remain elevated relative to the glazed-surface.

It has been found that the frits may be more conveniently applied by the wet process. Under this arrangement, the first frit, which matures into a glazed surface, is applied by dipping or spraying and then at least partially dried. The second frit is then applied upon the first frit in the desired pattern as, for instance, by spraying through a suitable stencil. The receptor thus coated is then dried in advance of firing.

During final firing, the first frit liquifies into a completely viscous state, and settles into a stratum somewhat reduced in thickness. Concurrently, the second frit partially liquifies. At this stage of the firing process, the flux of both frits liquify and amalgamate along a mutual margin designated by numeral 15, in Figure 3. It has been observed that the excess silica, or the like, of the second frit inhibits a portion of the viscous matter of both frits, when the final firing temperature is definitely lower than the temperature required to mature completely the second frit. This action is probably due to surface tension and cohesive force. Although the flux of the second frit liquifies, the higher melting point of the silica, and the difference between the coefficient of expansion of the two frits, operate to prevent the second frit from completely amalgamating with the molten first frit. Thus, the fired frits, although settled somewhat, mature into respectively glazed and matte surfaces, with the matte surface remaining elevated relative to the glazed-surface.

In Figure 3, the numeral 16 illustrates a fillet that forms adjacent the junction of the surfaces of both frits during firing. At this stage of the

firing process, firing is complete, and the receptor is removed from the furnace, while the second frit yet retains a dull or matte surface and remains in its relative elevated position.

5 Although the frits have been described as being fired simultaneously, it is also possible to apply, dry and fire the first frit before applying the second frit. Under this arrangement, firing for the second frit is carried out in the manner outlined above. Under these conditions, the glazed vitreous-enamel re-liquifies under the second or final firing to provide the required partial amalgamation of the frits as aforesaid.

It has been observed that silica, sand or the like may be employed in place of the second frit. Under this alternative, the silica is applied in the same manner described for the second frit, dried, and fired simultaneously or sequentially, as outlined above in connection with the two frits. It must be remembered, however, that the final firing temperature must be definitely lower than that which would liquify the silica, and at least equal to the temperature required to mature the first frit.

20 25 When using silica instead of a second frit, final firing is complete when the fillet 16 forms adjacent the junction of the surfaces of the two materials, as described hereinbefore in connection with the two frits. At this time the receptor is removed from the furnace, and it will be observed that the surface of the areas containing the silica have a fine granular-texture and remain elevated relative to the glazed enamel-surface.

30 35 From the foregoing, it will be apparent that the texture of the surface provided by the second frit, or silica, is largely dependent upon the proximity of the final firing temperature to the temperature required to mature fully the second frit, or silica, into a glazed-surface.

40 45 Accordingly, in order to provide the most effective "non-slip" floor-surface with a minimum total area for the "traction-spots," it is preferable to maintain the final firing temperature definitely lower than that required to mature the second frit, or silica, but at least equal to that required to mature the first frit into a glazed, vitreous-enamel surface. Also, the time of firing must be controlled, and the receptor removed from the furnace as soon as the first frit matures and the fillet 16 forms. This is important in order that the traction surface provided by the second frit, or silica, remains elevated relative to the surface of the glazed vitreous-enamel.

55 60 65 To produce the pattern illustrated in Figures 4 and 5, it has been observed that a wire screen or cord netting may be employed as a stencil, which stencil is placed directly on top of the first partially dried or fired frit, as described hereinbefore, and the second frit is preferably applied by spraying.

As illustrated in Figures 4 and 5, the latter arrangement provides a uniform distribution of relatively small pads of the second frit or silica, and, at the completion of the final firing, the floor surface has a plurality of uniformly distributed protuberances formed by the second frit remaining elevated relative to the glazed coating. 70 In this respect, it is to be understood that the arrangement illustrated in Figures 4 and 5 is shown on a greatly enlarged scale.

Having thus described my invention, I claim:

1. The method of producing a non-slip vitreous-enamel surface having unglazed areas ele-

vated relative to the remaining glazed area, comprising, applying to a base member a wet coating of vitreous-enamel material having a relatively low maturing temperature; at least partially drying the said material; applying upon portions of the surface of the so dried material, a wet vitreous-enamel material having a maturing temperature higher than that of the first applied material; firing the said materials at a temperature at least equal to the lowest maturing temperature but lower than the higher maturing temperature, to mature completely the material having the lower maturing temperature; and stopping firing as soon as the flux of the materials liquify and amalgamate at the junction of the surfaces of the said materials.

2. The method of producing a non-slip vitreous-enamel surface having unglazed areas elevated relative to the remaining glazed area, comprising, applying to a base member a first frit having a relatively low maturing temperature; applying upon portions of the surface of the said first frit, a second frit having a relatively high maturing temperature; firing the said frits at a temperature between the maturing temperatures of the said frits to mature completely the said

first frit; and stopping firing as soon as the flux of each of the said frits amalgamate and form a fillet at the junction of the marginal edges of the elevated second frit with the surface of the first frit.

3. The method of producing a non-slip vitreous-enamel surface having unglazed areas elevated relative to the remaining glazed areas, comprising, applying to a base member a first frit having a relatively low maturing temperature; applying upon portions of the surface of the said first frit, a second frit having a relatively high maturing temperature and in sufficient quantity so that its surface is elevated relative to the surface of the first frit; firing the said frits at a temperature between the maturing temperatures of the said frits and at least equal to the liquifying temperature of the flux of each frit, so as to mature completely the first frit and liquify the fluxes of each frit; and stopping firing as soon as the liquified flux of the first frit amalgamates with the liquified flux of the second frit to bond the unmatured second frit upon the surface of the matured first frit in its elevated relation relative thereto.

CHARLES T. GORDON.